

## UNITED STATES PATENT OFFICE

2,373,158

## BRASS POWDERS

John Wulff, Cambridge, Mass.

No Drawing. Application December 28, 1943,  
Serial No. 515,986

11 Claims. (Cl. 75—0.5)

This invention relates to the production of improved brass powder particularly adapted for powder metallurgy.

The usual method of making so-called bronze powder consists essentially of beating an alpha brass into very thin leaves then screening, grading and polishing the product. This is a protracted operation since the material is successively treated in different and progressively lighter stamps with intermediate screening between each stamping operation. In all such operations the starting material consisted of true alpha brasses, i. e., solid solution copper zinc alloys containing no more than about 36% zinc.

The present invention stems from a new concept in the fabrication of brass powders, namely, the concept of utilizing a special starting material which is characterized by a much higher degree of brittleness than the alpha brass, positively utilizing such brittleness to insure rapid disintegration and subsequently annealing the disintegrated product under conditions which insures controlled dezincification. The product thus produced is comprised of particles which have a high zinc content core and a lower zinc exterior or case of desirable plasticity which renders the powder readily amenable to pressing. When employed for powder metallurgy purposes such powder is pressed and sintered. As will be seen the sintering operation may be controlled readily so as to insure diffusion of the zinc from the zinc-rich core into the case or exterior to insure a substantially uniform distribution of the zinc with minimum evaporation or sublimation of the zinc.

The salient novel features of the process will be appreciated more readily from a consideration of a typical method which embodies the principles of the invention. The starting material for the process comprises an alpha-beta brass, i. e., a brass composed of alpha brass and a substantial amount of the embrittling beta constituent. As source material, therefore, there may be used any brass containing above about 36% zinc such for example as "Muntz" metal. The starting material may be derived from any suitable scrap which has been cleaned thoroughly.

To insure the best and standard results it is advisable to start with a melt. In carrying out the invention a brass melt is made containing a sufficient amount of zinc to positively insure the presence of the beta constituent in the alloy. In a typical case the melt may contain approximately 50% of copper and 50% of zinc by weight.

The melt may be suitably deoxidized, as with phosphorus, in the usual manner. The molten alloy is then immediately transformed into discrete solid particles. This may be done in any desired manner as by shotting or atomizing.

The product thus produced, as will be appreciated, is essentially a brittle alloy. This is then crushed to the desired particle size distribution. This may be done by disintegrating 10 in any suitable unit such as a ball or hammer mill, pneumatic attrition mill and the like. The crushed material may then be classified into the desired screen fractions. The several fractions may be blended or admixed in the proportions desired to give a predetermined particle size distribution.

The powder so produced is subjected to a controlled heat treatment the purpose of which is to distill off a predetermined amount of zinc and 20 to soften as well as brighten the powder. Preferably this is done by annealing in hydrogen. The annealing temperature should be above 500° C. and preferably about 800° C. Depending upon the zinc content of the original alloy the annealing time is controlled so as to distill off from about 10% to about 20% or more of zinc. The control may be such as to remove sufficient zinc so that the overall or residual zinc content is 36% or less, that is to say, so that the ultimate product is an alpha brass. The degree of dezincification, as will be appreciated, will depend upon the ultimate use to which the final sintered product is to be put. As those skilled in the art know the alpha brasses are progressively harder, and 25 stronger as the zinc content is increased up to about 35%. The ductility increases up to about 20% zinc and then falls. Thus, for products where ductility is of paramount or marked importance it may be desirable to carry out extensive dezincification so as to insure about 20% in 30 the final product.

As will be appreciated, the annealing may be effected in a closed system in which means are provided for recovering the zinc which may be 35 reused in subsequent melts. During the annealing operation the powder should be agitated so as to prevent sintering or cohesion of the particles.

The powder thus produced is constituted of 40 individually distinct particles which have a zinc-rich interior or core and a zinc-poor exterior case. The exterior or case, being relatively low in zinc is soft or plastic and thus amenable to ready deformation which is desirable in pressing. In making up powder metallurgy compacts the

powder is pressed at from about 15 to 35 tons per square inch and is sintered at a temperature under about 850° C. During the sintering operation the zinc diffuses into the zinc-poor case or exterior and thus tends to redistribute to give a substantially homogeneous alloy. It is particularly to be observed that a marked advantage of utilizing such a preheated brass powder, i. e., one with a zinc-poor ductile case is that there is much less tendency for the zinc to evaporate or sublime from the exterior denuded areas during the sintering operation.

The principles of the invention have been described utilizing as an example a simple case, i. e., one involving a binary alloy of copper and zinc. It will be understood that the invention may similarly be utilized in the production of powder metal compacts of ternary or other poly-nary alloys. Thus, the method may be employed to produce compacts of manganese bronze powder. In this case scrap metal can be used as the basis for the melt and zinc may be added to bring it up to approximately a 1 to 1 ratio with copper. Other metals may be used as addition agents in the melt to confer their respective effects on the ultimate alloy. Thus, additions of about 4% manganese, 2% iron, 1.5% lead, 1.5 to 5% aluminum and up to 2% tin may be desirable for certain end-products. As is known within certain limited ranges lead improves the machinability of brass; manganese and aluminum enter into solid solution in the alpha brass and increases its strength; iron tends to decrease grain size and increases the tensile strength, likewise iron as well as manganese and nickel usually improves the corrosion resistance of these brasses. It will be understood therefore that the invention is of broad application and is applicable not only to the binary brass alloy but to what for the sake of a term, may be called a brass base alloy, i. e., one containing minor percentages of the enumerated or other alloying constituents whose particular effect is desirable.

While a preferred embodiment of the invention has been described it is to be understood that this is given didactically to illustrate the underlying principle of the invention, i. e., the utilization of a relatively high percentage of one constituent so as to insure inherent brittleness and concomitant easy and rapid disintegration to a desirable particle size followed by removal of a predetermined amount of such constituent to render the exterior of the particles more plastic and pressable and then pressing and sintering under conditions which insure a diffusion of the constituent outwardly of the core to secure a substantially uniform composition in the ultimate product.

I claim:

1. A powdered brass comprising particles consisting of a core of brass of a relatively high zinc content and an integral case of a lower zinc content.

2. A powdered brass particularly suitable for the production of powder metal compacts which

comprises individually distinct particles of brass having a relatively brittle core and a relatively ductile case.

3. A method of producing powder metal compacts which comprises, shotting an alpha-beta brass melt, disintegrating the shotted material, annealing the disintegrated material under conditions regulated to insure the removal of a predetermined percentage of zinc largely from the exterior surface of the disintegrated particles and to render such surfaces plastic, pressing the annealed material and sintering the pressed material at a temperature and for a period of time sufficient to insure substantial diffusion of zinc to said exterior surfaces.

4. A pressable brass powder for powder metallurgy purposes comprising individual particles having a core of an alpha-beta brass and an internal case of alpha brass.

5. A pressable brass powder for powder metallurgy purposes comprising individual particles having a relatively brittle core of an aluminum-containing alpha-beta brass and a relatively ductile external case of an aluminum-containing alpha brass.

6. A pressable brass powder for powder metallurgy purposes comprising individual particles having a relatively brittle core of a manganese-containing alpha-beta brass and a relatively ductile external case of a manganese-containing alpha brass.

7. A method of producing brass powders which comprises shotting a brass melt containing more than about 36 percent zinc to produce a brittle shot; disintegrating the shot and annealing the shot under conditions regulated to distill off a predetermined percentage of the contained zinc.

8. A method of producing brass powders which comprises shotting a brass melt containing more than about 36 percent zinc to produce a brittle shot, disintegrating the shot, annealing the disintegrated shot under conditions regulated to distill off a predetermined percentage of zinc and recovering the distilled zinc.

9. A method of producing brass powders which comprises shotting a brass melt containing more than about 36 percent zinc to produce a brittle shot, disintegrating the shot and annealing the disintegrated material in hydrogen at a temperature between 500° C. and 800° C.

10. A method of producing brass powders which comprises shotting a brass melt containing more than 36 percent zinc to produce a brittle shot, disintegrating the shot and agitating and annealing the material under conditions regulated to distill off a predetermined percentage of zinc.

11. A method of producing brass powders which comprises shotting a brass melt containing more than about 36 percent zinc to produce a brittle shot, disintegrating the shot and annealing the material in hydrogen at a temperature between 500° C. and 800° C. and agitating the material during the annealing operation.

JOHN WULFF.